

# United States Patent Office

2,846,401  
Patented Aug. 5, 1958

1

2,846,401

## GRANULAR DETERGENT COMPOSITIONS

Thomas M. McCarthy and Arvid S. Roald, Cincinnati, Ohio, assignors to The Procter & Gamble Company, Cincinnati, Ohio, a corporation of Ohio

No Drawing. Application June 28, 1956  
Serial No. 594,365

9 Claims. (Cl. 252—138)

The present invention relates to anionic detergent compositions which are free-flowing and resistant to caking, and more particularly to spray dried, heavy-duty, phosphate-containing, anionic synthetic detergent compositions which possess improved stability against caking, lumping, and the development of a non-free-flowing character during storage under humid atmospheric conditions. The invention also relates to the process of producing such detergent compositions.

Among the commercial heavy-duty synthetic detergent compositions well known in the art, are spray dried mixtures of water soluble anionic synthetic detergents of the sulfuric reaction product type with massive amounts of alkali metal tripolyphosphate. Such detergent compositions, for example, are disclosed in detail in U. S. Patent 2,486,922 to Strain. Particularly efficient compositions, for example, are the spray dried products which are based on the sodium salt of alkyl sulfuric acid esters of higher alcohols obtained by the reduction of tallow and coconut oil and those which are based on sodium polypropylene phenyl sulfonate with 9-18, and preferably with 12-15 carbon atoms in the polypropylene chain, and mixtures thereof. In general, such compositions are commercially available in the form of solid spray dried granules whose components fall within the following percentage ranges: from about 20% to about 40% by weight of active synthetic from about 10% to about 60% by weight of alkali metal phosphates, such as sodium tripolyphosphate, pyrophosphate and orthophosphate, the latter two phosphates being present usually as a result of reversion of tripolyphosphate during spray drying, but sometimes being deliberately added, from about 10% to about 30% by weight of sodium sulfate, and from about 5% to about 25% of miscellaneous ingredients, which can include, for example, moisture, perfume, carboxymethyl cellulose, coloring and fluorescent dyes, organic builders, sodium silicate, and other inorganic alkaline salts.

The tendency of such detergent compositions to cake upon prolonged storage, particularly in areas of high humidity and high temperature, is known and numerous efforts have been made to overcome this tendency. Moisture-proof containers of special and expensive construction to guard against penetration of moisture laden air have been suggested. Special silicate formulas and other materials have been proposed as anti-caking agents for incorporation in the composition prior to spray drying. Moreover, admixture of the spray dried granules with steam or water to promote substantially complete hydration of hydratable components in the spray dried particles has been advocated. These methods of treatment have met with some measure of success, but they do not offer the complete solution to the product characteristic problems that are encountered in practice.

For example, under storage conditions in southern coastal areas where high temperature and high humidity prevail for extended periods of time, the prior art methods

2

of manufacture may reduce the tendency for the spray dried products to solidly cake in the carton, but they do not produce a composition which retains its free-flowing characteristic after storage for appreciable periods of time at 75% relative humidity and 90° F. for example. Under such conditions of temperature and humidity, the detergent particles, even after water treatment to reduce the content of unhydrated inorganic salts, have been observed to develop a tendency to hang together or to adhere to each other or to bridge or lump and, in general, to show a reluctance to flow freely as distinguished from the freshly produced granules.

In the course of the investigation of this problem, examination of products possessing free-flow reluctance as above defined, has revealed that this undesirable property is apparently caused by needle-like crystals which rapidly develop at about 75% relative humidity and about 90° F. and which tend to grow and radiate from the individual granules. Crystals having lengths up to 2 or 3 times the granule diameter have been noted. By intermeshing or by actual inter-granular crystal growth, a plurality of granules can become physically connected, thus affecting the free-flowing characteristics of the product. In the course of further study, such needle-like crystals were isolated and subjected to qualitative micro analysis. It was found that the crystals were intermediate hydrates of a mixture of trisodium and acid sodium orthophosphates. This was later confirmed by X-ray diffraction pattern analysis. While such phosphates may be purposely included in heavy-duty polyphosphate-containing detergent compositions of the nature of those herein disclosed, more frequently they result either from partial reversion of tripolyphosphate during the spray drying step or from hydrolysis of tripolyphosphate during storage subsequent to water or moisture treatment of the granules.

It is an object of the present invention to provide improved heavy-duty synthetic detergent compositions of improved free-flowing character and noncaking properties.

Another object is to provide heavy-duty synthetic detergent phosphate-containing washing compositions which have superior resistance to change in caking and free-flowing characteristics when subjected to storage for prolonged periods of time at relatively high temperature and high humidity.

Another object is to provide an improved heavy-duty synthetic detergent composition which does not require expensive moisture-proof containers for storage under humid atmospheric conditions.

A further object of the invention is to provide a process for the production of the above noted improved heavy-duty detergent compositions.

The present invention is directed to the solution of the problem of development of free-flow reluctance during storage under certain conditions of humidity and comprises agitating spray dried particles of heavy-duty synthetic detergent compositions hereinbefore referred to and simultaneously applying to the surface thereof an aqueous solution of a sulfate of magnesium, zinc, aluminum, or mixtures of such salts. The amount of solution applied to the particles is selected so that the concentration of inorganic sulfate salt applied to the granules ranges from about 1% to about 10% of the weight of the granules treated, preferably from about 2% to about 4%. The concentration of the inorganic sulfate in the solution applied to the granules is not critical, and can be adjusted within a range of 10% by weight to saturation, a concentration of about 18% to 22% by weight being preferred, so that the desired amount of magnesium, zinc, or aluminum salt, per se can be applied to the granules while at the same time the moisture content of the granules is increased from the normal of about 5% to 10% content to

an amount within the range of about 12% to about 25%, preferably from about 14% to about 17%.

The temperature conditions under which the aqueous solution of sulfate salt is applied to the granules is not critical, but of course reasonable limits should be observed. For example, the invention has been practiced by applying the solution to granules at ordinary room temperature from about 70° F. to about 90° F. and at temperatures such as those occurring at the base of the conventional spray drying tower, that is, from about 160° F. to about 200° F. Higher and lower temperatures can also be used, but care should be exercised to produce a product having a moisture content within the aforementioned range. Thus, the amount of moisture evaporation that may take place during transfer or cooling of the granules by air-lift will bear consideration.

It has been noted that the application of the magnesium, zinc, or aluminum sulfate, or mixture of such salts, in accordance with the invention not only imparts marked resistance to the development of free-flow reluctance in the granular product, but also surprisingly achieves a resistance to true caking that is far superior to that noted in products whose granules have been treated with water alone.

Investigation has indicated that the inorganic sulfate salt enters into chemical reaction with granular components at substantially the surface of the particles, thereby, for example, forming low or nonhydrating double salts with the phosphates, and especially those phosphates resulting from the reversion or hydrolysis of tripolyphosphate, i. e., orthophosphates and pyrophosphates. Thus, the needle-like crystals of orthophosphate which lead to free-flow reluctance and hydrates of other phosphates which lead to caking are not formed when the treated product is exposed to humidity and temperature conditions conducive to the development of the undesirable characteristics herein mentioned.

Investigation has also shown that the anion of the inorganic salt is important in achieving optimum results and that the sulfates of magnesium, zinc, and aluminum are markedly superior to other soluble salts of these metals such as the chlorides and acetates, which are no more efficient than water alone.

The specific method whereby the inorganic salt solution is applied to the spray dried granules does not constitute a part of the invention and the solutions may be applied continuously or batchwise as may be desired. In the normal operation of spray dried detergent granule production, the dried and cooled granules are usually passed continuously through a rotating drum where they are tumbled. The drum may be equipped with plates or baffles affixed to the inner wall thereof to provide more effective tumbling. It is conventional to mix the spray dried granules in such a rotating drum apparatus with ingredients such as perfume, organic builder, or other desirable adjuncts that might be volatilized or thermally decomposed under the more elevated temperature conditions occurring within the spray-drying tower. Magnesium, zinc, or aluminum sulfate solution designed for treatment of the spray dried particles in accordance with the present invention can be applied to the particles in such conventional rotating drums, either simultaneously or sequentially with the application of other constituents by spray-on procedure. Other methods of application of the solution to the granular particles are known in the art and can be employed without departing from the spirit of the invention.

The invention will be fully understood from the above description and especially when taken in conjunction with the specific examples which follow.

#### Example I

100 parts of spray dried detergent granules containing 28% sodium polypropylene benzene sulfonate in which the polypropylene radical averaged about 12 carbon

atoms, about 19.5% sodium tripolyphosphate, and about 13% sodium pyrophosphates, about 1.5% sodium orthophosphates, about 6% sodium silicate solids having a ratio of  $\text{SiO}_2 : \text{Na}_2\text{O}$  of 2:1, about 7.2% moisture, about 2.4% ethanolamide of mixed coconut oil fatty acids, and the balance being mainly sodium sulfate with minor amounts of carboxymethyl cellulose, fluorescent dyes and perfume, were agitated in a rotating drum and sprayed with a water solution of magnesium sulfate having a concentration of approximately 20%. The amount of anhydrous magnesium sulfate applied to the granules amounted to about 2.5% and the moisture content of the treated product was increased to about 17.3%. This product was packaged and stored under temperature and humidity conditions which were known to promote free-flow reluctance and caking. The product was found to be resistant to the development of free-flow reluctance and even after fourteen days of storage was as free-flowing and free from caking as the initial product.

It is believed that the magnesium sulfate in the solution sprayed on the granules reacts with the pyro- and orthophosphates at or near the surface of the granules to form low hydrating or nonhydrating magnesium-sodium phosphates. This belief has been supported by evidence which indicates that the equilibrium moisture of the granules containing the sprayed-on magnesium sulfate decreases with increasing amounts of magnesium sulfate. If, in the product of this example, the magnesium sulfate did not react with any component of the granules, it would form its heptahydrate and an increase in equilibrium moisture would be expected. Thus, the product of this example and the products of the invention in general are characterized by a coating comprising hydrated double salts of the phosphates formed from sodium and from the magnesium (or zinc or aluminum) of the magnesium sulfate solution applied.

#### Example II

In the manner described in Example I, 100 parts of the same spray dried detergent granules were treated with a solution of aluminum sulfate of approximately 20% concentration so as to coat the particles with about 2% anhydrous aluminum sulfate and to increase the moisture content to about 14.1%. The product so treated was packaged and stored under humidity and temperature conditions known to cause the development of free-flow reluctance and caking. The product was entirely resistant against the development of free-flow reluctance and was outstandingly resistant to caking.

A solution containing a mixture of aluminum sulfate and magnesium sulfate at about 20% concentration can also be employed in the place of the aluminum sulfate solution of Example II to yield a product having superior stability against caking and the development of free-flow reluctance.

#### Example III

The process of Example II was repeated using a solution of zinc sulfate of about 20% concentration. The resulting granular product, onto which was sprayed about 2% anhydrous zinc sulfate, had a moisture content of about 14.2% and was at least equal to the product of Example II in its stability against caking and the development of free-flow reluctance during storage under relatively high temperature and high humidity conditions.

#### Example IV

The treatment of detergent granules as specified in Example II is followed using a magnesium sulfate solution of approximately 20% concentration and a spray dried synthetic detergent composition containing about 35% sodium polypropylene benzene sulfonate in which the polypropylene radical averaged 12 carbon atoms, about 15.0% sodium tripolyphosphate, about 22% sodium pyrophosphates, about 2% sodium orthophosphates, about 6% sodium silicate solids having a  $\text{SiO}_2 : \text{Na}_2\text{O}$

ratio of 2:1, about 8% moisture, and the balance being mainly sodium sulfate with minor amounts of carboxymethyl cellulose, fluorescent dyes, and perfume.

Treatment of the granules so as to apply thereto approximately 2% anhydrous magnesium sulfate and to increase the moisture content to about 15% renders the product especially stable against caking and the development of free-flow reluctance during storage under atmospheric conditions of high temperature and high humidity.

The process of Example IV can also be applied to spray dried synthetic detergent granules which contain substantially greater amounts of sodium tripolyphosphate, such as from 1 to 1½ times the amount of active synthetic detergent and with smaller proportions of other phosphates, and the superiority of the products against the development of free-flow reluctance and caking under humid storage conditions is readily apparent.

In place of the polypropylene benzene sulfonate synthetic detergent used in the above examples, the sodium salt of the alkyl sulfuric acid esters of higher alcohols derived by the reduction of coconut oil or tallow can be substituted in whole or in part to yield products having superior characteristics as regards caking and freedom of flow.

Having thus described the invention, what is claimed is:

1. The process of improving the resistance to change, during storage under humid atmospheric conditions, in the free-flowing and non-caking character of freshly spray dried granular detergent compositions consisting essentially of a water soluble anionic synthetic detergent of the sulfuric reaction product type and hydratable alkali metal phosphates consisting essentially of a mixture of tripolyphosphate, pyrophosphates, and orthophosphates, which comprises agitating said spray dried granules and simultaneously spraying on the surface thereof an aqueous solution containing at least one inorganic sulfate of a polyvalent metal selected from the group consisting of magnesium, zinc, and aluminum, in amount equivalent to from about 1% to about 10% of anhydrous inorganic sulfate based on the spray dried granules and sufficient to raise the moisture content of the composition to an amount within the range of about 12% to about 25%.

2. The process of claim 1 in which the anionic synthetic detergent is, at least in substantial part, sodium polypropylene benzene sulfonate in which the polypropylene radicals average about 12 carbon atoms.

3. The process of claim 1 in which the amount of in-

organic sulfate solution applied is equivalent to an amount of anhydrous inorganic sulfate within the range of about 2% to about 4% and is sufficient to raise the moisture content of the granules to an amount within the range of about 14% to about 17%.

4. The process of claim 3 in which the inorganic sulfate is magnesium sulfate.

5. The process of claim 3 in which the inorganic sulfate is zinc sulfate.

6. The process of claim 3 in which the inorganic sulfate is aluminum sulfate.

7. The process of claim 3 in which the concentration of the inorganic sulfate solution is in the range of about 18% to about 22% by weight.

8. A spray dried heavy-duty synthetic detergent granule possessing improved resistance to change, during storage under humid atmospheric conditions, in the free-flowing and non-caking character of the freshly spray dried granule detergent compositions, consisting essentially from about 20% to about 40% by weight of water soluble anionic synthetic detergent of the sulfuric reaction product type, from about 10% to about 60% by weight of alkali metal phosphates including sodium tripolyphosphate and the pyrophosphate and orthophosphate reversion products thereof, from about 12% to about 25% moisture, and from about 10% to about 30% by weight of sodium sulfate, said granules being characterized by a coating comprising hydrated double salts of said phosphates formed from sodium and from at least one polyvalent metal selected from the group consisting of magnesium, zinc, and aluminum, the amount of polyvalent metal present being equivalent to an amount of anhydrous sulfate of said metal within the range of about 1% to about 10%.

9. The product of claim 8 in which the amount of polyvalent metal present is equivalent to an amount of anhydrous sulfate of said metal within the range of about 2% to about 4% and in which the amount of moisture is within the range of about 14% to about 17%.

#### References Cited in the file of this patent

#### UNITED STATES PATENTS

2,768,095 Tadema et al. ----- Oct. 23, 1956

#### FOREIGN PATENTS

974,713 France ----- Oct. 4, 1950

676,449 Great Britain ----- July 30, 1952